

## UNITED STATES PATENT OFFICE.

JOHN WENDELL ANDREWS, OF CHICAGO, ILLINOIS, ASSIGNOR TO WESTERN ELECTRIC COMPANY, INCORPORATED, OF NEW YORK, N. Y., A CORPORATION OF NEW YORK.

## METHOD OF PRODUCING MAGNETIC MATERIALS.

No Drawing. Application filed March 16, 1927, Serial No. 175,947. Renewed July 7, 1928.

This invention relates to methods of producing magnetic materials, and more particularly to methods of producing brittle magnetic alloys for use in electrical signaling apparatus, such as cores for loading coils employed in telephone circuits.

The principal object of the invention is the production of a magnetic material, having a fine crystalline structure, to facilitate its reduction to a very finely divided form, and possessing to a high degree those physical, electrical and magnetic properties which make it highly desirable in electrical signaling apparatus, especially in cores for loading coils for telephone circuits.

The magnetic material produced in accordance with the invention is of particular advantage in the production of magnet cores of the so-called "dust" type in which a magnetic material is reduced to very finely divided particles, the particles treated to produce an insulating coating thereon and pressed into rings or cores. One method of utilizing the finely divided magnetic material to produce loading coil cores is described in the copending application, Serial No. 102,729, filed April 17, 1926, by J. W. Andrews and R. Gillis. However, the magnetic material is not limited in its use to the particular insulator disclosed in the foregoing application nor to any particular form of core, but may be put to any use within the scope of the appended claims.

In accordance with one embodiment, the present invention contemplates the production of brittle alloys of nickel and iron by partially oxidizing the constituent metals while in the molten state and working the metal in the solid state, while hot, to produce a fine crystalline structure. More specifically, the invention contemplates the production of brittle nickel iron alloys, generally known as "permalloy" in which the proportions of its constituents are more than 25% nickel and the remainder principally iron, one form which has proven satisfactory, having a nickel content which is approximately 80% of the whole.

In this embodiment the constituents are melted in an uncovered furnace in the presence of oxygen and an oxidizing substance, the molten material is boiled until it is oxidized, is poured into a mold and allowed to solidify. The solidified material is then rolled while hot until it cools below the

temperature of recrystallization, which is indicated by a tendency to break in the rolls, when it is given an additional pass through the rolls to effect an additional reduction in order to produce a fine crystalline structure. 60

One method of oxidizing the metals constituting the alloy is disclosed in the copending application, Serial No. 101,179, filed April 10, 1926, by C. P. Beath and H. M. E. Heinicke, but for the sake of completeness 65 it will also be described in detail herein.

The method of producing the brittle, fine grained material in accordance with the invention consists in placing the required quantities of nickel and iron in an uncovered furnace, preferably electrically heated, adding a calculated quantity of oxidized material of the same purity, and heating the material until it is molten. The melting is done in an uncovered furnace in order that 70 the material may be oxidized by atmospheric oxygen. Since, if virgin metal is used, it requires considerable time to obtain a melt which is oxidized to the right degree, oxidized material may be added to furnish additional oxygen to reduce the time consumed in completing the operation. Iron oxide in the form of iron ore may also be added to furnish oxygen within the bath. When the material has become molten it is oxidized by 75

boiling for a length of time determined by the amount of oxidation desired and the type of furnace used. The degree of oxidation of the material depends upon the length of the melting period, the length of the boiling period, the amount of the surface of the melt exposed to the air, and the amount of oxygen present in the charged material, and the heating and boiling periods are governed by the various charges and the type of furnace used. Experiments have shown that the metal of a melt which is not sufficiently oxidized is not sufficiently brittle. Consequently to insure the exact amount of oxidation, the melt is heavily oxidized and a small 80 quantity of a suitable deoxidizer, such as magnesium-nickel alloy, aluminum or chromium, may be added just before the melt is poured. After the molten material 85

has been boiled the required length of time, it is then poured into an ingot mold, and as soon as the material is solidified, the mold is removed and the ingot is allowed to cool.

Samples of the material are taken from various parts of the ingot which are an- 90

alyzed, and if the material is of the required composition it is placed in a furnace where it is heated to approximately 1325° C., at which temperature it may be easily rolled.

- 5 In order to obtain a fine dust, the material should have a very fine crystalline structure, which is obtained by successively passing the hot billets from the heating furnace, without a subsequent reheating, through 10 progressively reducing rolls until the material has cooled to a temperature below its temperature of recrystallization, which experiments have shown to be at about the temperature at which the material becomes 15 "cold short", that is, the temperature at which the material breaks very readily when struck. The material is then broken into short lengths which are fed between rolls placed more closely together than any in the 20 prior series which effect a further reduction in the thickness of the material and at the same time effect a further reduction in the crystalline structure of the material.

The working of the metal breaks down the 25 large grained, crystalline structure of the billet and produces a very fine grained crystalline product which is extremely brittle. Since the final reduction in the size of the crystal is effected at a temperature below 30 the temperature of recrystallization of the material, the crystals do not grow in size after the final rolling and the resulting product has an extremely fine crystalline structure which is very desirable because in 35 this material the fracture takes place principally along the crystalline boundaries and consequently the finer the grain structure the finer the dust which can be produced from the finished product.

40 The short pieces obtained by the above operations are crushed in a jaw crusher, hammer mill, or any other suitable type of apparatus, after which the crushed material is rolled in a ball mill until it is reduced to 45 a fine dust. The dust is sieved through a 120 mesh sieve and any residue is remelted and carried through the above operations to again reduce the material to a finely divided form.

50 By using an alloy of the proportions stated in the preceding paragraph and by following the foregoing method of procedure, a very fine grained crystalline product is obtained which is extremely brittle 55 and which when reduced to a fine dust yields a large percentage of particles which are small enough to pass through what is commonly known as a 200 mesh sieve. When reduced to a finely divided form, the 60 material is then in a form to be used for either continuous or lump loading of telephone circuits.

The method of producing a magnetic material having a very fine crystalline structure is also applicable for use with magnetic

materials which have been rendered brittle by the addition of metallic embrittling agents such as antimony, tin, etc., and which have the property of fracturing principally along the crystal boundaries. If mechanical 70 work, such as rolling, is performed upon such alloys at temperatures slightly below their respective temperatures of recrystallization, the resulting materials will have very fine crystalline structures and may be 75 readily reduced by any suitable means to a finely divided state.

The finely divided magnetic material obtained by the above described methods is particularly adapted to be formed into rings 80 or cores for loading coils in any suitable manner. In one method which has proven satisfactory the finely divided particles are heated to a high temperature, are individually insulated by treating the particles in such a manner as to produce an insulating coating around each particle, the insulated material formed into rings or cores by the application of a high pressure, and the rings annealed to stabilize the insulator and 85 to give the rings the desired magnetic properties. A plurality of rings thus formed are then stacked coaxially to form a core on which the usual toroidal winding is applied, the number of such rings used depending upon the existing electrical characteristics of the telephone circuit with which the loading coils are to be associated. Since, in order to have low losses in loading 90 coil cores made of permalloy dust in the above described manner, it is desirable that all of the material pass through a 120 mesh sieve and a large percentage pass through a 200 mesh sieve, it is readily seen that the material produced according to this invention 95 is especially adapted to be used in the production of such cores.

What is claimed is:

1. The method of preparing magnetic materials which fracture principally along the crystal boundaries thereof, which consists in working the material at a temperature slightly below its temperature of recrystallization to produce a fine crystalline structure, and subsequently reducing the 110 material to a finely divided form.

2. The method of making magnetic materials, which consists in treating a magnetic material to render it brittle and working the material at a temperature below its 115 temperature of recrystallization to produce a fine crystalline structure.

3. The method of making magnetic materials, which consists in treating a nickel-iron alloy with an embrittling agent, and rolling the resulting material after it becomes "cold short" to effect a change in 120 the crystalline structure.

4. The method of making brittle magnetic materials, which consists in partially 125

oxidizing a magnetic material and working the material after it becomes "cold short" to produce a fine crystalline structure.

5 5. The method of making brittle magnetic materials, which consists in partially oxidizing a magnetic material and working the material at a temperature below the temperature of recrystallization to effect a 10 change in the crystalline structure.

6. The method of making brittle nickel-iron alloys, which consists in partially oxidizing the constituents and working the alloy at a temperature below its temperature of recrystallization.

7. The method of making brittle magnetic alloys, which consists in partially oxidizing a nickel-iron alloy while in the molten state, allowing the material to solidify 20 and rolling the material while hot until it has reached a temperature below its temperature of recrystallization.

8. The method of making brittle ferrous magnetic alloys, which consists in partially oxidizing the constituents, rolling the alloy 25 while hot until it becomes "cold short",

and then carrying the material through an additional rolling operation.

9. The method of making brittle magnetic alloys composed of more than 25% 30 nickel and the remainder principally iron, which consists in melting the ingredients in the presence of oxygen, boiling the ingredients until oxidized, allowing the resulting alloy to solidify, and rolling the alloy at a 35 temperature below its temperature of recrystallization.

10. The method of preparing magnetic materials in finely divided form, which consists in melting approximately 80 parts of 40 nickel and 20 parts of iron in the presence of oxygen, boiling the molten material until oxidized, allowing the resulting alloy to solidify, rolling the alloy while hot until it has reached a temperature below its temperature of recrystallization, and subsequently reducing the material to finely divided particles.

In witness whereof, I hereunto subscribe my name this 4th day of March A. D., 1927.

JOHN WENDELL ANDREWS.